

June 19, 1934.

F. L. LA QUE

1,963,137

PROCESS OF DYEING SILK CONTAINING TEXTILES

Filed Dec. 31, 1930

*Fig. 1.*



*Fig. 2.*



INVENTOR.

*Francis Lawrence La Que,*

BY  
*Bynes, Stellens, Parmenter & Blenko.*

ATTORNEYS.

## UNITED STATES PATENT OFFICE

1,963,137

PROCESS OF DYEING SILK CONTAINING  
TEXTILES

Francis Lawrence La Que, East Orange, N. J., assignor to The International Nickel Company, Inc., New York, N. Y., a corporation of Delaware

Application December 31, 1930, Serial No. 505,693

2 Claims. (Cl. 8—5)

The present invention relates to processes of dyeing textiles and more particularly to processes of dyeing silk material with dyestuffs of the sulphoncyanin type.

In the degumming and dyeing of silk and silk mixtures with dyestuffs of the sulphoncyanin type, there has been a tendency to non-uniformity of color in the dyed silk and particularly there was a tendency for each apparatus or dyeing machine to give a different amount of reduction of a dyestuff like Durol black (sulphon-cyanin black, Color Index Number 307), a common dyestuff used extensively in the dyeing of silk hosiery. Attempts have been made to overcome the non-uniformity in results of the dyeing operation. Various suggestions have been proposed but no proposal has been made which remedies the shortcomings of the prior practice. Under these conditions, it was necessary for the dyer to manipulate the dyeing formula to accommodate the peculiarities of each dyeing machine. This procedure has been unsatisfactory, has been costly and has required extensive and tedious experimentation each time a new machine was used and each time, during the life of a machine, when the peculiarities thereof have a tendency to change. This latter phenomenon has been one of common occurrence.

I have discovered a process which overcomes the disadvantages noted hereinabove and which provides the art with a process which can be satisfactorily and readily employed for producing uniform and consistent results.

It is a further object of the invention to provide a process in which the silk gum or serecin is prevented from detrimentally affecting the dyestuff and the dyeing of the silk or other fibre with which it is associated.

It is another object of the invention to provide a process which will dye silk material with sulphoncyanin uniformly and without any material variation in the shade or depth of color of the dyed material and to provide a machine for carrying this process into practice.

Other objects and advantages of the invention will become apparent from the following description taken into conjunction with the accompanying drawing in which:

Fig. 1 is an elevational view of a dyeing machine embodying the present invention; and

Fig. 2 is a side elevation of Fig. 1.

Generally speaking, the present invention contemplates maintaining a sufficient concentration or supply of oxygen in the dyeing bath to prevent reduction of the dyestuff, such as sulphon-

cyanin, by the serecin or silk gum, or other substances present in the dyeing vat. In practice, it is preferred to introduce oxygen by means of bubbling, blowing or otherwise causing air to be brought into the dyeing bath and to agitate the latter to effect substantially uniform distribution of the air throughout the dyeing bath. When this procedure has been followed, it has been found that the dyeing operations such as the dyeing of hosiery with sulphoncyanin, can be carried out satisfactorily and can be effected so as to produce silk or hosiery dyed to the proper shade or depth of color.

The foregoing procedure can be conveniently and satisfactorily carried into practice by the use of a dyeing machine such as illustrated in the drawing.

Referring more particularly to Fig. 1, the reference character 10 designates an outer drum, preferably of cylindrical construction and mounted upon side frames 11. This side frame may be of any suitable construction but as herein shown being constituted of two upright members 12 and a bottom cross member 13. The upper part of outer drum 10 is provided with a sliding door 14 which can be opened when textiles such as silk material or silk socks are introduced into the drum or when inspection is made and closed when the dyeing machine is in operation.

Within outer drum 10, is mounted an inner cylinder 15 of open character. This cylinder may be supported for rotation in any suitable manner as by means of stub shaft 16 extending through each end of the dyeing machine as one skilled in the art will readily understand. As the construction of the inner cylinder is well known, it will not be necessary to give a detailed description thereof. It is sufficient to state that the inner cylinder is so constructed that textiles such as silk hosiery can be introduced into and taken from the cylinder in any suitable manner.

The inner cylinder is driven by a prime mover such as an electrical motor 17 through any suitable driving mechanism. In the present instance, a train of driving gears are employed. For instance, gear 18 on the motor drives an intermediary gear 19, which in turn drives a gear 20 that is keyed or otherwise suitably secured to shaft 16. These gears are preferably housed in a gear guard 21. The driving mechanism may be arranged to drive the inner cylinder continuously in one direction or can be arranged to periodically alternate the rotation of the cylinder.

At one end of the dyeing machine a valved steam line 22 is connected to the outer drum for

introducing steam into the dyeing machine to maintain the dyeing bath at a proper or suitable temperature. Preferably adjacent to the steam line is a pipe 23 which conducts solutions such as degumming or dyeing or both from supply tank 24 to the interior of the outer drum 10. A valve 25 serves to control the flow of liquid from tank 24 to drum 10.

Arranged in operative association with the dyeing machine are means for introducing oxygen or air into the dyeing bath held in outer drum 10. Any appropriate means may be employed for effecting the introduction of oxygen or air into the dyeing bath. In the present instance, an elongated pipe 26 is provided in the outer drum 10 and preferably near the bottom thereof. This pipe is perforated and permits air or oxygen to be bubbled into the dyeing bath. An appropriate source of air or oxygen may be utilized for supplying pipe 26 with oxygen or air. For example, an air blower 27 is connected to pipe 26 for supplying air thereto and is driven by motor 28. A valve 29 is provided on pipe line 26 to control the amount of air being blown into the dyeing bath contained in outer drum 10.

In carrying the invention into practice, the dyeing and degumming bath to be employed is placed in outer drum 10. For instance, a solution of Durol black or sulphoncyanin is introduced into drum 10. The textiles or textile material such as silk hose are introduced into inner cylinder 15 and the dyeing machine is set into operation. The air blower is operated and a controlled amount of air is introduced into the dyeing bath. When the silk hose is properly dyed without any substantial reduction in color or depth of shade, the proper amount of air has been added. This test can be conducted very easily and readily before the process is started.

In practice, it is preferred to saturate the solution with air or oxygen because in this manner sufficient oxygen will be present to bring about the desired results of this invention. Any excess air or oxygen does not cause any detrimental effects.

It has been found that in dyeing silk hose, for example, with sulphoncyanin and using a degumming solution having a pH of about 9.3 to about 9.8 and a temperature of about 200° F. to 215° F., sufficient air to saturate the solution with oxygen was satisfactory. By controlling the aeration device to supply sufficient oxygen or air to the dyeing bath to saturate the same, reduction of the dyestuff can be prevented under

substantially any practical conditions. With my process, degumming can be effected at the same time the silk is dyed. By introducing sufficient air or oxygen into the degumming and dyeing bath the temperature of the latter may be increased to a sufficient degree to enable degumming to be effectively carried out. In the same way by saturating the bath with air or oxygen, degumming solutions of higher pH values can be used with more effective degumming.

It is preferred to construct the dyeing machine and parts thereof which come into contact with the silk and dyeing bath of such materials which are inert to the dyestuff employed for dyeing the silk. For example, it is preferred to construct the machine of a nickel-copper alloy in which the nickel varies from about 60% to about 70% and the copper varies from about 40 to about 30%. Other appropriate metals which do not detrimentally affect the dyeing of silk may be employed.

Although certain preferred temperatures, pH values and oxidizing agents were mentioned, it is to be understood that the invention is not limited thereto. For instance, other appropriate oxidizing agents may be used in place of air and oxygen such as ozone or solid compounds capable of liberating oxygen and satisfactorily effecting the results described herein. Other variations and modifications may be made without departing from the scope and spirit of the invention.

What is claimed is:

1. In the process of dyeing silk material, that improvement which comprises establishing a degumming and dyeing bath having a pH value of about 9.3 to about 9.8 and containing Durol black, heating said bath to a temperature in excess of about 200° F., and blowing air into said bath to prevent the reduction of Durol black.
2. In the process of degumming and dyeing silk hosiery material, that improvement which comprises establishing a degumming and dyeing bath of about 9.3 to about 9.8 and containing Durol black, heating said bath to a temperature of about 200° to about 215° F., introducing silk hosiery material into said bath, maintaining said bath at a temperature in excess of 200° F. and blowing air into said bath to saturate the same and to prevent the reduction of Durol black, whereby the silk hosiery material is dyed to the proper shade.

FRANCIS LAWRENCE LA QUE.